

## UNITED STATES PATENT OFFICE

2,513,788

## BLEACHING OF SULFATE WOOD PULP

George A. Day and Benjamin G. Hoos, Berlin,  
N. H., assignors to Brown Company, Berlin,  
N. H., a corporation of Maine

No Drawing. Application January 31, 1947,  
Serial No. 725,722

1 Claim. (Cl. 8—106)

**1** This invention relates to the bleaching of cellulosic materials, particularly wood pulp.

One object of the invention is to produce highly bleached wood pulps, both sulphate and sulphite, of exceptional physical characteristics heretofore unobtainable by known bleaching methods.

A further object of the invention is to produce, by less complicated, quicker or less costly treatment, bleached pulps having physical qualities equivalent and even superior to those now obtained.

Bleached pulps produced in accordance with this invention may have brightnesses of 88, 89, 90 (General Electric reflectance value) and higher, with beater values as great as those of the unbleached pulp, indicating substantially no degradation of the fiber during treatment. The bleaching treatment of this invention is so effective that exceptional bleached sulphate pulp physical values, not ever attained heretofore in five-or-six-stage sequences, may be secured, oftentimes in as few as three stages; and normal sulphite pulp values of five-or-six stage sequences may very readily be attained in three stages.

In the practice of this invention, chlorine dioxide is utilized as a bleaching reagent under novel and unusual conditions productive, in the case of this reagent even in a single stage, of remarkable jumps in brightness value without loss in other physicals.

While the treatment herein described may be applied as a late or final stage in any pulp bleaching sequence, for realization of the highest physical values in the novel sulphate pulps of this invention, particularly brightness and beater values, the sequence includes hot (140–210° F.) caustic digestion as one stage preparatory to chlorine dioxide treatment and preferably a combination pretreatment, prior to the hot caustic digestion, of pre-bleach and chlorination, wherein the amount of bleaching reagent input (calculated as equivalent chlorine) in the pre-bleach is from 20–50% of the total equivalent chlorine input of the entire sequence.

The chlorine dioxide treatment in accordance with this invention is carried out under stock density conditions of 4% or less, at a pH of  $6 \pm 1$ , and at a temperature of at least 140° F.

Typical treatments are as follows:

*Example I (sulphate)*

A softwood kraft pulp was pretreated with 5.5% chlorine at a stock density of 4% for 2 hours at 65° F., and then was washed.

It was then digested with 1½% NaOH at 14.5% <sup>55</sup>

**2** stock density for 2 hours at 140° F., and then washed.

As a third and final stage, the pulp was subjected at a stock density of 4% and at a pH of 5.8 to the action of 1.19% chlorine dioxide based on the bone dry pulp (the chlorine dioxide containing from 3 to 8% chlorine as an impurity) at 180° F. for 2 hours, and then washed, antichlored with SO<sub>2</sub> water and again washed.

10 The bleached pulp had the following physical characteristics:

|                                                 |      |
|-------------------------------------------------|------|
| Brightness (General Electric reflectance value) | 89.3 |
| 15 Beater value (2 × Mullen (136) + Tear (306)) | 578  |

This beater value equalled the beater value of the raw pulp, which was likewise 578.

*Example II (sulphate)*

A softwood kraft pulp was subjected to the action of 8% hypochlorite bleach at 8% stock density and 75° F. for one hour and was then diluted, without intervening washing, to 4% stock density with sufficient chlorine water to give 2.7% chlorine, based on the weight of the bone-dry pulp, and maintained for one hour at 65° F. and then was washed, antichlored with SO<sub>2</sub> water and again washed.

20 30 As a second stage, the pulp was then subjected to a hot caustic treatment with 1.5% NaOH at 14.5% stock density for two hours at 140° F. and then washed.

As a third and final stage, the pretreated pulp was subjected at a stock density of 4% to the action of 0.95% chlorine dioxide based on the bone-dry pulp (the chlorine dioxide containing from 3 to 8% chlorine as an impurity), at pH 5.8 and 180° F. for two hours and then washed, antichlored and again washed.

40 The bleached pulp had the following physical characteristics:

|                                                 |      |
|-------------------------------------------------|------|
| Brightness (General Electric reflectance value) | 91.0 |
| Beater value (2 × Mullen (140) + Tear (308))    | 588  |

This beater value again equalled the beater value of the raw pulp which was 588.

50 In this sequence, the initial bleaching agent input, calculated as equivalent chlorine was 35% of the total equivalent chlorine input for the three stages. It has been determined that highest values are attained in the case of pre-bleach treatment of this kind where the pre-bleaching,

i. e., the hypochlorite chlorine equivalent input is from 20 to 50% of the total equivalent chlorine input in the entire sequence. For example, use of 59.8% of the equivalent chlorine input in the hypochlorite pretreatment on the same stock in a sequence otherwise identical with that of Example II, resulted in a reduced brightness value of 88.2 and beater value of 557. Further increase to 73% reduced brightness to 85.2 and beater value to 535.

*Example III (sulphite)*

A sulphite raw stock of 17.3 Tappi permanaganate number was subjected to the action of 5.5% chlorine at 4% stock density, 65° F. for 30 minutes, then washed.

The washed pulp was next treated with 1% NaOH at 4% stock density, 65° F. for 15 minutes and then thickened to about 16 to 18% stock density.

As a final stage, the pretreated pulp was subjected to the action of 0.85% chlorine dioxide based on the bone-dry pulp (the chlorine dioxide containing from 3 to 8% chlorine as an impurity), at a pH of 6.2 and a stock density of 4% at 180° F. for two hours and then washed, antichlorosed with SO<sub>2</sub> water and again washed.

The bleached sulphite pulp had the following physical characteristics:

Brightness 88.5  
Beater value 2×Mullen (127) + Tear (168) 422

This compared with a raw stock beater value of 408, and a beater value only 387 (117 Mullen; 153 Tear) for the same raw stock bleached by identical first stage and caustic soap treatments followed by a customary present-day third stage treatment with 6.5% soda bleach, 0.75% NaOH at 10% stock density for almost six hours at 110° F. to 89.0 brightness.

The brightness values above given for kraft pulps of this invention exceed those secured by the customary present-day treatments when the strength of the raw pulp is maintained. Present-day kraft pulp having brightness values even as high as 86 are obtainable only by five, six or more stage bleaching sequences, whereas the above kraft pulps are the result of three-stage treatment.

The preferred kraft pulps of this invention have beater values exceeding 550, and, as above disclosed, ranging as high as 578 or more, while maintaining brightness values above 88 and even as high as above 90.

With the sulphite pulp, it will be noted that this process yields a bleached pulp with exceptionally high beater value and high brightness,

the beater value of the bleached pulp being higher than the beater value of the raw pulp. In general, with sulphite pulps beater values of the bleached pulp will be higher or at the least substantially as high as that of the raw pulp and exceed 420 even when bleached to brightness as high as 88.

Whereas the chlorine dioxide treatment, as given in the above examples, calls for treatment for two hours at 180° F., a range of 140–180° F. is suitable, varying with the time of treatment.

While the examples hereinabove given are for novel pulps of this invention of almost spectacular physical characteristics, it is to be understood that the treatment hereof is applicable to any pulp to give increased bleaching efficiency even in the production of pulps of conventional lower brightness values in the range down to 80.

We claim:

Process of bleaching sulphate wood pulp which consists in treating the pulp sequentially, without intervening washing, with hypochlorite and chlorine, the equivalent chlorine input on the treatment with hypochlorite being from 20–50% of the total equivalent chlorine input of the entire process, then digesting the pulp with caustic soda at a temperature between 140° F. and 210° F. and finally treating the pulp in aqueous suspension with chlorine dioxide, said final treatment being carried out at a temperature of at least 140° F., at a stock density not exceeding 4%, and at a pH of 6±1.

GEORGE A. DAY.  
BENJAMIN G. HOOS.

REFERENCES CITED

The following references are of record in the file of this patent:

UNITED STATES PATENTS

| Number    | Name    | Date           |
|-----------|---------|----------------|
| 2,129,719 | Vincent | Sept. 13, 1938 |
| 2,166,330 | Vincent | July 18, 1939  |
| 2,228,127 | Richter | Jan. 7, 1941   |
| 2,377,171 | Murdock | May 29, 1945   |
| 2,408,849 | Haney   | Oct. 8, 1946   |

FOREIGN PATENTS

| Number  | Country       | Date          |
|---------|---------------|---------------|
| 191,357 | Great Britain | Mar. 22, 1923 |
| 567,774 | Great Britain | Feb. 3, 1945  |

OTHER REFERENCES

Jahn, Modern European Pulp Bleaching, Paper Trade Journal, Sept. 20, 1945, Tappi Secs., pages 113–115.